

Sept. 6, 1927.

1,641,479

D. FINLEY

METHOD OF TREATING PAPER BOARD

Filed June 13, 1923



Fig. 1

Fig. 2



Fig. 3



Fig. 4



Fig. 5

Fig. 6

INVENTOR.  
DOZIER FINLEY  
BY *White Root & Evans*  
ATTORNEYS.

Patented Sept. 6, 1927.

## UNITED STATES PATENT OFFICE.

DOZIER FINLEY, OF BERKELEY, CALIFORNIA, ASSIGNOR TO THE PARAFFINE COMPANIES, INC., OF SAN FRANCISCO, CALIFORNIA, A CORPORATION OF DELAWARE.

## METHOD OF TREATING PAPER BOARD.

Application filed June 13, 1923. Serial No. 645,088.

The invention relates to the production of paper board of a water-proof and grease-proof character, and one of the objects of the invention is the production of a paper board, processed with paraffine, which during the process undergoes a minimum of discoloration or a controlled discoloration. Another object of the invention is the provision of a process whereby a paraffine treated paper board or paper board articles of handsome appearance may be produced from a relatively inexpensive grade of paper board.

Another object of the invention is the provision of a process of paraffining paper board which may be carried out without painstaking control of temperature and the chilling bath, and which produces a more brilliant, and in the case of white coated board a whiter product, than is possible by former methods. A further object is the conservation of the more valuable materials used in producing this general class of paper board.

Other objects of the invention together with the foregoing will be set forth in the following description of the preferred process and the means for practicing the same, which is illustrated in the drawings accompanying and forming part of the specification. It is to be understood that I do not limit myself to the showing made by the said descriptions and drawings, as I may adopt variations of my preferred form within the scope of my invention as set forth in the claims.

Referring to the accompanying drawings: Fig. 1 is a sectional view of a piece of board of my invention. The view is largely diagrammatic and certain portions have been emphasized out of their true proportion in order to make the structure clear. Fig. 2 illustrates diagrammatically one method of carrying out the operations involved in my invention and Fig. 3 illustrates another method. Fig. 4 is a plan view of a piece of my paper board illustrating a decorative effect, which it is possible to secure in the practice of my invention. Fig. 5 illustrates diagrammatically an apparatus by which the decorative effect shown in Fig. 4 may be secured, and Fig. 6 is a side elevation of one of the rolls forming part of such apparatus.

In the making of many types of paper board packages, popularly known as cartons, it has been the custom to cost the paper

board with paraffine wax, preferably melting at about 130° Fahrenheit, and applied in the molten state by a variety of methods which are well understood and need not be explained here. The thickness of the paraffine coating adds about two-thousandths of a millimeter to the thickness of the paper board, and this is divided between the two sides. Not all of the paraffine is superficially coated upon the boards. Some of it soaks into the boards to a slight extent. A paper board comprising a straw colored filler and a white liner and having a thickness of approximately nine-thousandths of a millimeter when paraffined, shows a mottled effect, proving that the paraffine has penetrated the thinner part of the liner sufficiently to render it translucent. A board having twice the thickness of white liner will not show this mottled effect. This is indicative of a penetration of paraffine ranging between six and twelve-thousandths of a millimeter.

If the board, just previous to the application of paraffine, is wet with water and then superficially dried it will be found that there is a diminished penetration of the paraffine as indicated by no evidences of discoloration. It is difficult, however, to control the wetting of the board so as to secure uniform results. If the board is too wet there is the possibility that the paraffine will not adhere to the surface, and if too dry penetration of irregular character will result.

I have found that if the board is wet with water containing dissolved gums, sugars or salts, a more even control is obtained. In such a case all of the water employed may be permitted to evaporate and a film of the previously dissolved matter is left on the surface of the board. This film is sufficient to reduce or prevent penetration of the melted paraffine into the outer structure of the paper board. It should be noted that it is not necessary to dry the board thoroughly before the paraffine is applied. In fact, in a continuous process it is preferable that the thorough drying out of the water be not sought, or that drying be obtained only so far as permitted by the limitation imposed by continuous operation.

A solution for treating the paper board which I have found very satisfactory comprises the following materials: 12 gallons of

water, 20 pounds sodium chloride, 27 pounds saccharose, 54 pounds glucose (from starch), 3 pounds sodium borate. The solution will be found to be just short of a syrupy consistency and to contain practically half water and half solids. It may be applied to the surface of paper board by saturating a cloth with the solution and rubbing the solution wetted cloth over the paper board which is then allowed to dry. When dry or practically dry, the board may be passed into a paraffining machine of known type and given a coating of paraffine over the solution treated surface. This method is suitable for a small amount of the paper board but on a large scale I prefer to follow one or the other of the following methods.

*First method.*—This method is especially adapted to the treatment of paper board on which discoloration is to be prevented on only one side, and is essentially a discontinuous process.

The board is first passed thru a set of rolls and given a paraffine treatment on the side on which discoloration is of no importance. This is the ordinary operation familiarly known as "paraffining one side." The board is now passed thru a set of rolls as illustrated diagrammatically in Fig. 2, in which the lower portion of a rubber covered roll 3 lies in a solution 4, prepared according to the above formula and contained in a pan 6. The roller 7 is adjustably held by well known means in such position above and relative to the roll 3, that only enough of the solution is permitted to be deposited on the board 8 to make the board wet and tacky to the touch without being flood coated. The greater part of the excess solution taken up from the tank 6 by the roller 3 is kept back by the doctor or scraper 9 thus protecting the roll 7 from becoming wet. A further protection for the same purpose is furnished by the doctor or scraper 11.

In the practice of my invention I have found that quantities ranging around  $\frac{3}{4}$  of an ounce of solution per square yard are sufficient, varying of course according to the porosity of the surface of the board. Sheets of board thus treated may be stacked or piled one on top of the other, although still wet on the solution treated sides, and the same applies to board which is treated in the roll, that is, it may be rolled up on a spindle without danger of sticking. Although the solution in drying becomes tacky or sticky it will not adhere to the contiguous paraffine coated surface. It will usually be found that the solution becomes dry in the time the board is stacked or rolled up. This is due to the water distributing itself thru the body of the board, and being held hygroscopically by the fibers, while the salts and gums and sugars of the original solution remain as a film on the surface of the board.

The board as treated in the above described process is next passed thru a second paraffining operation by which the solution treated side is coated with paraffine. It is obvious that paraffining may be on one or both sides. 1. on both sides, the paraffine of the first treatment is not appreciably augmented by the second treatment since it is largely remelted and displaced in part by new paraffine and in part remains in situ.

It will of course be appreciated that the board may be dried by evaporation of the water of the solution if the sheets are spread out singly or if they are put into or passed thru a drying chamber.

*Second method.*—The second typical process for carrying out the invention is practiced with an apparatus illustrated in Fig. 3. This is essentially a continuous process, and is adapted to the treatment of one or both sides of the board with the solution. This apparatus includes two sets of wringer rolls, one set comprising the rolls 13 and 14 and the other set comprising the rolls 15 and 16. The lower rolls 14 and 16 are partially immersed in the above described solution 17 contained in pans 18 and 19 respectively. Each of the rolls is provided with a doctor or scraper 21 to prevent excess solution being carried upwardly from the tanks upon the boards. The top rolls 13 and 15 are also provided with doctors or scrapers 22, and supply spouts 23 suitably valved are provided for carrying solution to the upper rolls. Preferably all the rolls are of rubber and are geared to run in the direction indicated. Means well known in the art are provided for adjusting the relative position of the rolls in each set and resiliently retaining the rolls in relative position by spring-pressed bearings.

The sheet of board 26 passing between the rolls, and coated on each side with a film of the solution, is received on a carrier belt 27, which passes over a heating coil or means 28. The hot air currents from the heating means help to evaporate the moisture from the solution on the board passing above. From the carrier belt 27 the board passes between the paraffining rolls 30, where it receives a film of the melted paraffine in a manner which will be understood by those skilled in the art. From the paraffining rolls the sheet passes into the water filled chilling tank 31 where the paraffine which has just been applied by the rolls is suddenly chilled so that a glazed finish is produced, without that crystallization which causes a more or less milky appearance.

In Fig. 1, I have shown in diagrammatical form and somewhat exaggerated, a section of paper board treated by my process. The body of the board 35 has been given a coating or film of the solution which has dried and left a residue 36 of the soluble materials

carried by the solution deposited on and saturated into the surface of the board. Over the solid material deposited on the board a thin film 37 of paraffine imparts a glazed finish to the board, which is both grease and water resisting. It will be noted that the paraffine layer 37 is not shown as having penetrated into the board and because of this lack of penetration no discoloration or 10 mottled effect occurs.

In Fig. 4 I have shown a plan view of a piece of board in which predetermined areas of the surface have been coated with the solution referred to above, so that when the paraffine is subsequently applied, the lack of absorption of the paraffine over the treated areas and its absorption in the untreated areas give rise to a pattern or decorative effect, which cannot be secured otherwise except by means which it is not practicable to use. In the diagonal line or lattice pattern shown in Fig. 4 the areas 38 are the untreated areas, and the areas 39 are the untreated areas, the untreated areas absorbing the paraffine more or less and hence taking on a darker shade than the treated areas. Obviously, variation in these decorative effects is infinite and trade-marks and insignia suggestive of water marks as well as other designs in a wide variety may be thus applied in an attractive way.

In Figs. 5 and 6 I have shown in diagrammatic form an apparatus for applying my solution to secure a decorative effect. A 35 sheet of paper 41 passes between the rollers 42 and 43, the upper of which has a plain face, and the lower provided with a resilient water insoluble facing such as rubber, and having the desired design molded or otherwise arranged thereon in relief as shown in Fig. 6. Solution from the pan 44 is carried up to the roller 43 by means of the roller 45 which acts like an inking roller. The amount of solution provided on the roller 43 is controlled by the doctor 46 arranged adjacent the roller 45.

If desired, dyes of various colors and intensities may be added to the solution to secure an enhanced decorative effect.

As indicated in the above description a wide range of concentration is possible in the coating solution. Not alone is this influenced by the texture of the board to be treated but different concentrations may be used on the same board. As noted, a mere wetting of the board with water will prevent the undesirable soaking in of the paraffine although it does not permit the desired close control. In a broad sense it may be stated that the use of a fluid varying from water to a solution in which there is a concentration of 50% or more of solids, will effect the purpose of the invention. The upper limit of concentration appears to 60 be that at which the solution becomes too

viscous to work properly. However, with the application of more pressure upon the wringer rolls, the amount of even a very viscous solution applied to the surface of the board may be reduced to a workable 70 quantity.

The ingredients of the solution are also capable of variation within a wide range. Casein may be used in the solution, preferably the mildly alkaline soluble forms of 75 casein. Flour or preferably starch may be used, either in the cooked or uncooked state. So also molasses, dextrine, animal glue, and where alkali will not affect the board or the printing thereon in an undesirable manner, 80 silicate of soda may be used. Any of these materials may be mixed with water, or combinations of them may be mixed in water in any desired concentration not having too high a degree of viscosity. 85

Since paper board cartons are very largely used for the packaging of food stuffs, it is desirable that the ingredients of the solution used on them shall be nonpoisonous. The ingredients I have named in the preferred form of the solution are not only non-toxic but with the exception of borax are common ingredients of food stuffs. Borax is commonly used in the dextrine 90 paste for cementing the cartons, and is as well known perfectly harmless unless taken into the human system in considerable quantity. 95

Instead of sodium chloride, ammonium 100 chloride may be used in the proportion of about 2½% by weight in the solution. The distinctly saline taste of sodium chloride or ammonium chloride makes the solution distasteful to flies which might be attracted by the sweetness of a glucose and sugar solution. The sugar or saccharose is used because it is 105 a common ingredient of food stuffs, is relatively cheap, and is extremely soluble in water. Glucose is used because it inhibits the crystallization of the other ingredients 110 when the water evaporates and because it is common in food stuffs and is relatively cheap. The borax serves as a preservative to prevent fermentation of the sugars if the solution should be thinned to a point where 115 ferment could act.

I have found that other solutions than those having a water solvent may be used in carrying out my process. Among them may be mentioned nitro-cellulose solutions and all of the class of solutions having a base of nitro-cellulose and having admixtures of other substances, such as castor oil, gum camphor, and tung oil. While such solutions are relatively more expensive than the water solutions above described, yet an extremely small amount of the nitro-cellulose film is effective in stopping the absorption of the paraffine. 125

Instead of applying the solution in the 130

manner illustrated and described it may be applied to the board by means of spray nozzles or brush machines of well known form.

5 Under some conditions it may be desirable to employ fillers in the solutions, such as china clay, or whiting for the purpose of filling the pores in the surface of the board, to extend the solution, and to add whiteness or 10 opacity to the surface underlying the paraffine. It is not however desirable to use solutions which contain a filler on printed board or printed blanks, as the filler tends to obscure the printing. Usually I find it 15 inadvisable to treat the board previous to printing. It is possible to use the solution in all workable concentrations on board which has been printed and my process is especially intended to follow the printing 20 of the stock and immediately precede the paraffining operation. Following the first method herein set forth and allowing the

board to dry, or using the nitro-cellulose solution, it becomes possible and is in some instances advisable to print the board after, 25 instead of before treatment with the solution.

I claim:

1. The method of treating paper board which comprises applying thereto an aqueous solution of sodium chloride, saccharose, 30 starch glucose and sodium borate and subsequently coating the surface with paraffine.

2. The method of treating paper board which comprises applying thereto a solution made substantially in accordance with the 35 following formula: 12 gallons water, 20 pounds sodium chloride, 27 pounds saccharose, 54 pounds glucose, 3 pounds sodium borate and subsequently coating the surface with paraffine. 40

In testimony whereof, I have hereunto set my hand.

DOZIER FINLEY.